

## UNITED STATES PATENT OFFICE.

DUNCAN MACRAE, OF EAST ORANGE, NEW JERSEY, ASSIGNOR TO WESTINGHOUSE LAMP COMPANY, A CORPORATION OF PENNSYLVANIA.

## INCANDESCENT ELECTRIC LAMP.

No Drawing.

Application filed December 2, 1921. Serial No. 518,509.

My invention relates to the manufacture of incandescent electric lamps and more particularly to improving the quality of such lamps.

5 Incandescent electric lamps, especially of the vacuum type, having substantially pure tungsten filaments, are considerably improved for commercial usage by an operation known in the art as flashing. Briefly 60  
10 stated, this operation consists in lighting the lamp on a high resistance, high voltage circuit so designed that when the lamp is first lighted on this circuit a harmful flow of current will not take place within the lamp. 15  
15 By this preliminary treatment, the lamp is rendered fit for usage on a commercial circuit without danger of its destruction by arcing.

20 The accepted meaning of the term arcing as employed in the lamp industry, is the conduction of the current in the space surrounding the filament and the leading-in wires. An excessive amount of such conduction would affect the lamps to such an extent as 25  
25 to harm the normal operation thereof, and usually results in the complete destruction of the lamp.

According to modern electrical theories, 30 the conduction of the current in the space surrounding the filament and the leading-in wires takes place because of the presence therein of ions, i. e. charged particles which may consist of single electrons, charged atoms, or charged atom groups. According 35 to these theories, gas or vapor consisting of uncharged atoms or molecules will not conduct any current. However, under potential gradients very much greater in value than those which may exist in normally operating incandescent-filament lamps, gaseous molecules become ionized even between cold electrodes. It is also true that under the 40 potential gradients existing in normally operating incandescent-filament lamps, the electrons emitted by the filament will not cause the conduction of appreciable current in the evacuated lamp space. But when gaseous molecules and atoms arising from the decomposition of gas evolving substances 45  
50 or the interaction between the filament and such substances, at certain favorable pressures, ranging from a few thousands bars to about 100 bars, a bar being equivalent to about .00075 millimeters of mercury, surround incandescent filaments emitting elec-

trons, the potential gradient in normal operating lamps (especially those operating above 100 v.) is sufficient to cause the production of ions by the collision of rapidly moving electrons with the atoms or molecules. A sufficient number of ions may then be present to allow the conduction of a harmful amount of current through the space surrounding the filament. 60

In lamps as ordinarily constructed there exists after evacuation, pressures of from 2 to 50 bars of gas capable of being measured with a McLeod gauge. In addition to this, there is very probably an equal or greater quantity of water vapor the exact quantity 70 of which is not readily measured. Also when the filament is first lighted the number of molecules in the space surrounding it is temporarily increased by the effect of the filament temperature upon certain substances, known in the art as getters. These substances are introduced into the lamp to improve the efficiency of the lamp by removing residual gases and retarding the blackening of the bulb. An example of such 75  
80  
85

getters is a mixture of an inorganic halogen compound and phosphorous held on the filament by a binder of nitro-cellulose. When a lamp containing a filament coated with such a getter is first lighted, the number of molecules in the space surrounding the filament is considerably increased by the molecules resulting from the decomposition of the binder and the vaporization of the phosphorus and the inorganic halogen 90 compound. During this first lighting, the getter is said to be activated. In the example given, this activation consists in vaporizing it from the filament to the bulb, for during this transitory movement it encounters 95 the molecules of residual gas and carries them to the bulb walls and disposes the inorganic halogen salt in a transparent coating capable of retarding obscuration of the bulb by the evaporated particles of the filament. From the foregoing, it is evident in lamps as at present constructed that during activation of the getter or during first lighting of the lamp, pressures exist which fall within the limits set forth above, and 100 destruction of the lamp will result if it is lighted on a commercial circuit without resistance in series therewith to prevent the conduction of a harmful amount of current. 105  
110  
A specific example may be helpful in un-

derstanding the mode of treatment pursued under standard practices in vogue at the present time in the larger lamp manufacturing establishments. A 40 watt, 110 volt 5 Mazda B lamp, which, as is well known, is an evacuated lamp having a substantially pure drawn-tungsten filament coated with a getter usually comprising a mixture of cryolite and phosphorus affixed to the filament by a nitro-cellulose binder, is connected to a 330 volt circuit containing a resistance in series with the lamp somewhat greater than 550 ohms. This resistance, when the circuit is closed, is designed to prevent the 10 conduction of a harmful amount of current between the leading-in wires and the filamentary parts. It is evident that even if sufficient ions are present in the space surrounding the filament to conduct a current 15 sufficient to destroy the lamp, if burned on a commercial circuit, that on the circuit described no matter how low the resistance of the lamp, a current greater than .6 of an ampere, i. e., the applied potential of 20 330 volts divided by the resistance of 550 ohms, cannot flow through the filament and through the space surrounding the filament, and accordingly the current conducted by the gas will be much less than .6 of an 25 ampere. The flashing operation may continue for about one minute, and during this time the series resistance is successively replaced by smaller resistances until after removal of the residual gases sufficient current 30 is allowed to flow through the filament to raise its temperature slightly above that at which it is adapted to normally operate. During this flashing operation, the phenomena of the "blue glow" occurs and is 35 generally considered to indicate a successful removal of residual gases. As a result of this treatment the strength of the filament is reduced to the extent that occasionally 40 lamps are produced which will not withstand the shocks incident to transportation, which obviously results in a direct loss to the manufacturer as well as an inconvenience to the purchaser. This reduction, according to some authorities, is the result 45 of the attending heat treatment received by the filament.

Having in mind that it is probably the 50 heat treatment just described, to which practically all lamps are at present subjected, which produces the weakened condition in the filaments, I have discovered by 55 actual experiments, more fully referred to hereinafter, that such treatment may be considerably modified, or even entirely eliminated, by reason of which I have materially 60 improved the qualities of the lamp and overcome the results incident to heat-treatment under present practices. Furthermore, I have also discovered that the shrinkage 65 resulting directly from arcing and the

reduced filamentary strength resulting from the factory methods pursued in order to prevent the occurrence of arcs when the lamp is burned directly on a commercial circuit, may be entirely eliminated.

It, therefore, becomes an object of my invention to improve the quality of an incandescent lamp by effecting a reduction or elimination of the harmful effects resulting from the flashing or heat treatment given a lamp prior to shipment by the manufacturer thereof.

In determining to what extent the treatment could be modified to secure the desired ends, I conducted a series of experiments with a number of lamps containing filaments gettered with cryolite, which is one of the standard getters. The getter was affixed to the filaments in accordance with the method described in my application for patent, Serial No. 470,672, filed May 18, 1921, for a getter and method of applying the same and assigned to the Westinghouse Lamp Company. This method, briefly stated, differs from previous methods of applying the getter in that the getter substance is fused on the filament without the presence of organic compounds or phosphorus. These lamps were placed directly on a normal commercial circuit without having been previously burned. The lamps burned without the conduction of any harmful amount of current between the metal parts of the lamp, and indicated in most cases that insufficient current flowed through the space between the metallic parts of the lamp to show even the "blue glow" well known in the art. Despite contrary opinions, the vacuum obtained in such lamps as evidenced by the usual tests, was substantially equal to those in lamps in which the blue glow occurred.

A series of experiments were then performed in which I used a getter consisting of powdered glass, which, according to L. Hamburger in the Proceedings of the Amsterdam Academy of Sciences, vol. 21, p. 1074, possesses both the capacity of removing residual gases and nullifies the obscuration of the bulb by tungsten or filamentary particles. This getter substance was affixed to the filament by the fusion process described in my copending application identified above. These lamps, without previously having been burned, were burned directly on a normal commercial circuit without any appreciable resistance in series, and none of them arced.

From the foregoing experiments I concluded that the manner in which the getter substance is applied to the filaments has considerable to do with the prevention of arcing, provided good commercial exhaust is given the lamps. This is evident from the aforementioned experiments, as by fusing

the getter to the filaments the introduction of substances capable of evolving gases or which tend to promote ionization of the gases within the lamp or which are favorable to ionization, i. e., have a low ionizing potential, may be eliminated. Phosphorus and organic materials tend to remove any thin coating of oxide on the filament as well as to reduce the thorium oxide in the filament with the formation of thorium, a metal known to have a high capacity for emitting electrons, and thus allow greater freedom of electron emission. By thus reducing the causes which promote arcing, as explained more fully above, one of which being the introduction of gas-evolving substances with the getter, the flashing schedule to which the lamps are subjected in order to avoid this phenomenon occurring when first lighted on a commercial circuit, may be safely eliminated.

I further determined from a series of experiments conducted with several lamps gettered with cryolite and phosphorus affixed to the filaments thereof with a nitro-cellulose binder, which is in accordance with standard practice, which lamps were exhausted according to standard factory methods and thereafter flashed at 86% of the normal operating current which had been determined by experiment to be the minimum current for conditioning the lamp to burn on a commercial circuit, that no improvement was noticeable in the strength of the filament. However, in following up this line of experiments, I replaced the cryolite in the standard point getter given by a low-boiling getter substance, such as lithium fluoride, giving the lamps a slightly better exhaust than that obtained on the automatic machines at present in use in the factory. When thus treated, I found that during the flashing operation I could safely lower the flashing current employed from 86% of normal current to a current not greater than 72% of normal current. Bump tests conducted on these lamps after flashing at the 72% current, showed a marked increase in filament strength over that obtained with the lamps flashed at the 86% current. From these experiments I am inclined to believe that either the improved exhaust given the lamp or the lower melting-point getter used, which probably effected a removal of residual gases under conditions of voltage and filament temperature unfavorable to gaseous conduction of electrical current, or perhaps the combination of both these changes enabled me to lower materially the flashing current. Getter substances having high ionizing potentials are to be preferred. It is believed that this is a property of lithium fluoride.

Later experiments were carried out with a series of lamps gettered with a cryolite-phosphorus-nitro-cellulose binder mixture. These lamps were given a sufficiently good exhaust resulting in a final pressure of a few bars and involving a heating of the lamp for one minute at a temperature just insufficient to cause harmful softening of the glass lamp parts at substantially atmospheric pressure immediately before transference to the exhaust apparatus. It is probable that during the exhausting of the lamp, most of the phosphorus and the gases resulting from the nitro-cellulose binder, as well as any gases held by the finely divided cryolite, were removed from the lamp. These experiments confirmed my belief that by removing the media which are favorable to arcing, the lamp could be safely burned for the first time directly on a commercial circuit of the designed lamp voltage.

From the foregoing experiments and the careful analyses of the results secured thereby, I have concluded that by reducing the electrical conductivity of the space surrounding the filament and the leading-in wires, or by reducing such conductivity to a harmless amount, that the lamp may be rendered fit for safe initial burning on a low resistance commercial circuit.

Furthermore, in contradistinction to certain modern theorists, I find it unessential to treat the filaments of incandescent electric lamps before burning them on a commercial circuit in order to render them safe, and am convinced that even if such treatment is found desirable for inspection reasons or otherwise that the lamp can be burned in the factory at much reduced initial burning values, and if for any reason, it is desired to eliminate the present step of flashing in the fabrication of an incandescent lamp that this may be done and the lamp safely burned for the first time directly on a commercial circuit, at which time the getter substance may be activated.

I claim to have discovered that the electrical conductivity of the space surrounding the leading-in wires and the filaments may be controlled by regulating the composition and physical state of the getter material applied to the filament when the lamp has received a good commercial exhaust. Where the vacuum in a lamp is that obtained under the best operating exhaust conditions and substances capable of evolving gases or evaporating from the incandescent filament are not present in the lamp in harmful quantity, danger of arcing therein when the same is placed on a commercial circuit need not be feared. It will thus be seen that the preliminary flashing now accorded the lamp could be eliminated from the present steps pursued in the fabrication of a lamp and the cost of production correspondingly diminished. Furthermore, a lamp would be obtained whose fila-

125  
130

mentary strength is substantially unchanged and, therefore, since the original structure before burning is much stronger than that which obtains after burning, 5 lamps could be shipped and handled without any danger of shrinkage from that source.

I also claim to have discovered that if, for any reason, it is undesirable to eliminate flashing, as for instance, where a final inspection is preferred, that the original filament strength can be substantially maintained by reducing the lighting schedule or the current utilized in such 15 schedule to a value where the treatment accorded the lamp at that schedule will not be harmful to the strength of the filament. These experiments show that by employing a getter having a low boiling-point, the 20 object of flashing may be attained even in the presence of harmful gas-evolving substances at a temperature sufficiently low to materially reduce harmful effects to the filament.

25 I am aware of certain efforts which have been made in the past to eliminate the conduction of current in the space surrounding the metallic lamp parts or the so-called Edison effect in incandescent electric lamps, 30 but such efforts have not been extended to the prevention of such conduction when the vacuum type lamp is first lighted. On the contrary, however, this blue glow has been considered beneficial and serves as an indication of the removal of residual gases. 35 I am also aware of published articles in which mention is made that when certain getters are flashed the absence of any blue glow is observed. But, so far as I have 40 been advised, no one has hitherto considered the beneficial results which may flow from obviating this phenomenon.

Although I have specifically described 45 certain modes of treatment and the reduction in the number of factory operations at present employed, it is to be appreciated that modifications may be made which come within the scope of my invention as set forth in the appended claims.

50 What is claimed is:

1. The method of producing an incandescent electric lamp for use on a commercial lighting circuit without the necessity of previously flashing the same which consists in exhausting the lamp to a sufficient degree to render the residual gases substantially non-conductive at the rated voltage of the lamp and applying a getter to the filament which is activated on initial burning of the filament without evolving sufficient gases to produce appreciable positive ionization.

2. The method of producing an incandescent electric lamp for commercial use without previously flashing the same, 65 which consists in reducing the electrical conductivity of the space surrounding the leading-in wires and the filament by controlling the quantity and condition of the conducting media within such space by fusing the getter to the filament in said lamp.

3. An incandescent electric lamp of the vacuum type having a low residual gas content and an unactivated getter which on initial burning of the filament is completely 75 vaporized without the evolution of a harmful amount of permanent gas.

4. A commercially complete incandescent electric lamp of the vacuum type having an unburned filament therein.

5. A commercially complete incandescent electric lamp of the vacuum type having an unburned filament and an unactivated getter therein.

6. A commercially complete incandescent 85 electric lamp of the vacuum type having an unburned filament and an unactivated getter thereon capable of activation when the lamp is initially lighted upon a commercial circuit.

7. An incandescent lamp having a getter substance therein which on initial burning of the lamp is vaporized without the evolution of gases which harmfully conduct the current.

95 In testimony whereof, I have hereunto subscribed my name this 1st day of December, 1921.

DUNCAN MacRAE.